

# UNITED STATES PATENT OFFICE.

WILLIS R. WHITNEY, OF SCHENECTADY, NEW YORK, ASSIGNOR TO GENERAL ELECTRIC COMPANY, A CORPORATION OF NEW YORK.

## METAL-WORKING.

1,008,762.

No Drawing.

Specification of Letters Patent. Patented Nov. 14, 1911.

Application filed March 23, 1910. Serial No. 551,156.

To all whom it may concern:

Be it known that I, WILLIS R. WHITNEY, a citizen of the United States, residing at Schenectady, county of Schenectady, State of New York, have invented certain new and useful Improvements in Metal-Working, of which the following is a specification.

In the process of wire drawing, it is necessary to point, or sharpen, the ends of the rod or wire before each reduction, as it is of somewhat greater diameter than the die through which it is to be drawn.

My invention involves a process by which oxidizable metals, particularly metals of the chromium group, such as tungsten or molybdenum, are pointed expeditiously, leaving a clean surface free from pits or scars. My invention is of general application to the chemical removal, or corrosion, of these metals and can be used for other purposes, as for example, to clean dies accidentally plugged.

If it is desired to point a rod consisting of a metal of the chromium group, as for example, tungsten, the rod is dipped into a fused bath consisting of an oxidizing salt, preferably a bath consisting of a fused nitrite, such as potassium or sodium nitrite. The nitrite need not be pure. I find the commercial salt which ordinarily contains small amounts of impurities, such as chlorids, answers very well for the purpose. In some cases it is advantageous to heat the ends of the rod or filament before dipping into the fused bath, but it is usually sufficient to simply dip the rod or wire into the fused bath. In fact, the heat generated by the chemical action of the nitrite on the wire heats the wire to redness. If it is desired to clean a steel die plugged with tungsten, for example, the die is simply dipped into the fused nitrite and the tungsten is thereby dissolved out without any appreciable corrosion of the steel taking place. Other oxidizing baths, for example, the nitrate of sodium, or of potassium, can be used, but, in this case, a diluent, such as the chlorid of sodium

or potassium, or the hydroxid of either of these metals should be added, as the nitrate used by itself acts so vigorously that it tends to pit and roughen the surface of the metal.

What I claim as new and desire to secure by Letters Patent of the United States, is,—

1. The process of chemically removing all or a part of a body of a metal of the chromium group, which consists in bringing the body of metal into contact with a fused, oxidizing compound.

2. The process of chemically removing all or a part of a body of metal of the chromium group, which consists in bringing the metal into contact with a fused bath containing a nitrite.

3. The process of pointing a tungsten rod or wire which consists in dipping an end of said rod or wire into a fused nitrite.

4. The process of dissolving, or corroding, a solid body of tungsten which consists in bringing it into contact with a fused nitrite.

5. In the process of drawing tungsten, the step which consists in pointing the tungsten rod, or wire, by dipping it into fused potassium nitrite.

6. The process of dissolving, or corroding, a body of tungsten which consists in bringing it into contact with a commercial salt of nitrous acid maintained at an elevated temperature.

7. The process of corroding a body of metal of the chromium group which consists in acting upon it with a fused oxidizing compound containing a diluting substance inert with respect to said metal.

8. The process of chemically removing tungsten from a body of said metal which consists in bringing it into contact with a fused salt of an oxyacid of nitrogen.

In witness whereof, I have hereunto set my hand this 21st day of March, 1910.

WILLIS R. WHITNEY.

Witnesses:

BENJAMIN B. HULL,  
HELEN ORFORD.